

Patented Jan. 17, 1950

2,494,736

## UNITED STATES PATENT OFFICE

2,494,736

## COPPER BASE ALLOY

John D. Berwick, Alton, Ill., assignor to Olin Industries, Inc., East Alton, Ill., a corporation of Delaware

No Drawing. Application October 20, 1945, Serial No. 623,609

2 Claims. (Cl. 75—157.5)

1

This invention relates to copper base alloys and more particularly to such an alloy containing as essential constituents, copper, zinc, aluminum, and manganese.

A primary object of this invention is the provision of a relatively inexpensive alloy having strength characteristics, hardness and the like properties comparable to, or improved over, those of the usual aluminum bronzes, but having greatly improved working characteristics and particularly suited as a bearing alloy. The aluminum bronzes employed as a bearing metal heretofore known usually contain copper, aluminum and iron, with or without the inclusion of other elements such as zinc, nickel, lead, tin, manganese, and silicon. Such alloys require a relatively high annealing temperature between cold working operations in order that such cold working operations may be satisfactorily accomplished. It is therefore, an object of this invention to provide an alloy which may be relatively inexpensively hot or cold worked and which permits relatively low annealing temperatures between cold working operations and also relatively low temperatures for hot working. Another object is to provide an alloy which can be utilized to provide bearings having low resistance to friction combined with long wearing qualities.

The above and other objects are accomplished in accordance with this invention by the provision of an alloy having a composition within the limits of 80% to 89% copper, 4% to 15.5% zinc, 3.5% to 6.5% aluminum, and 1% to 2.5% manganese. A composition within the above limits containing 85.5% to 88.5% copper, 4% to 6.5% zinc, 5.5% to 6.5% aluminum, and 1.5% to 2.5% manganese is preferred, since this composition has higher strength and hardness with elongation and conductivity substantially equivalent to other compositions within the above limits, thus rendering it especially suited for automotive and aircraft bearings.

It has been found that the inclusion of substantially less than 80% copper in the alloy results in decreased ductility making cold rolling operations unsatisfactory. The inclusion of less than 3.5% aluminum results in an undesirable decreased strength and hardness, whereas aluminum contents higher than about 6.5% result in casting difficulties and in the precipitation of a delta phase, materially reducing the ductility. More than about 2.5% manganese materially lowers the conductivity whereas less than about 1% manganese results in an undesirable lower strength and hardness. The manganese component contributes greatly to lower the temperature required for annealing after cold working

operations. The zinc component improves the hardness and less than about 4% zinc makes casting of the alloy difficult. Minor amounts of impurities such as iron or lead are permissible without destroying the desirable properties of the alloy.

The physical properties of typical compositions exemplifying this invention are shown below in comparison with the properties of a typical prior 10 aluminum bronze alloy containing iron as an alloying element. Alloys of this invention are designated by the letters A, B, C, D, and E, and the prior alloy is designated by the letter F.

TABLE 1

## Composition

|                       | A    | B    | C              | D    | E    | F    |
|-----------------------|------|------|----------------|------|------|------|
| Copper.....percent    | 87.3 | 87.5 | 80.1           | 87.5 | 88.4 | 87.0 |
| Zinc.....do.....      | 5.2  | 6.2  | 15.2           | 6.7  | 5.8  | 7.0  |
| Aluminum.....do.....  | 5.8  | 4.0  | 3.6            | 4.2  | 3.6  | 4.0  |
| Manganese.....do..... | 1.7  | 2.3  | 1.1            | 1.6  | 2.2  | —    |
| Iron.....do.....      |      |      | Less than 0.1  |      | 2.0  | —    |
| Lead.....do.....      |      |      | Less than 0.05 |      | 0.03 | —    |

TABLE 2

## Physical properties

[After cold rolling to 50% reduction—no subsequent anneal]

|                                             | A     | B     | C     | D     | E     | F     |
|---------------------------------------------|-------|-------|-------|-------|-------|-------|
| Tensile Strength 1000 p.s.i.                | 118.7 | 116.0 | 117.7 | 112.0 | 114.0 | 112.0 |
| Elongation percent in 2 inches <sup>1</sup> | 2.0   | 1.0   | 1.0   | 1.0   | 3.0   | 3.5   |
| Hardness (Rockwell B)                       | 96.5  | 94.0  | 94.0  | 93.0  | 95.0  | 95.0  |

<sup>1</sup> Test specimen 0.5 in. wide by 0.020 to 0.080 in. thick.

TABLE 3

## Physical properties after annealing

|                                             | A    | B    | C    | D    | E    | F    |
|---------------------------------------------|------|------|------|------|------|------|
| Anneal Temp., °C.....                       | 575  | 575  | 575  | 575  | 650  | 720  |
| Tensile Strength 1000 p.s.i.                | 69.0 | 66.0 | 67.8 | 62.2 | 58.0 | 67.5 |
| Elongation percent in 2 inches <sup>1</sup> | 45   | 41   | 43   | 46   | 65   | 42   |

<sup>1</sup> Test specimen 0.5 in. wide by 0.020 to 0.080 in. thick.

TABLE 4

## Electrical conductivity

|                                 | A    | B    | C    | D    | E    | F    |
|---------------------------------|------|------|------|------|------|------|
| Conductivity, Percent IACS..... | 12.5 | 11.0 | 13.0 | 12.0 | 11.5 | 13.6 |

It may be seen from Table 3 that the alloy of this invention permits an annealing temperature substantially less than 600° C., whereas the prior alloy F requires an annealing temperature substantially above 700° C., in order to obtain about the same physical characteristics suitable for subsequent cold working. It may be seen that composition E when annealed at a temperature as high as 650° C. had a tensile strength much lower and a percent elongation much higher than prior composition F which was annealed at the temperature of 720° C., thus further demonstrating the fact that the alloy of this invention permits a much lower annealing temperature than such prior alloys. It should also be noted that the preferred composition containing 85.5% to 88.5% copper, 4% to 6.5% zinc, 5.5% to 6.5% aluminum, and 1.5% to 2.5% manganese, as exemplified by composition A, Table 1, has a materially higher hardness, Table 2, with elongation and conductivity, Table 4, substantially equivalent to the other compositions, rendering it especially suitable for a bearing material. The alloy of this invention, in addition to providing advantages in cold working operations, likewise permits the use of a lower temperature for hot working operations than is ordinarily employed with prior aluminum bronzes, which is of decided advantage, since an economy in heating is effected and greater reductions in thickness of metal are permissible between heating operations.

Thus, in accordance with this invention a novel ductile alloy having high strength and hardness and other properties such as low resistance to

friction and grabbing necessary to produce good bearings is provided.

Having thus described the invention, what I claim and desire to secure by Letters Patent is:

1. A copper-base alloy susceptible to annealing at relatively low temperatures between cold working operations composed of 4% to 15.5% zinc, 3.5% to 6.5% aluminum, 1% to 2.5% manganese, and the balance copper, the copper content being 80% to 89%.

2. A copper-base alloy susceptible to annealing at relatively low temperatures between cold working operations composed of 4% to 6.5% zinc, 5.5% to 6.5% aluminum, 1.5% to 2.5% manganese, and the balance copper, the copper content being 85.5% to 88.5%.

JOHN D. BERWICK.

#### REFERENCES CITED

The following references are of record in the file of this patent:

#### UNITED STATES PATENTS

| Number    | Name     | Date          |
|-----------|----------|---------------|
| 1,764,034 | Palm     | June 17, 1930 |
| 1,848,858 | Webert   | Mar. 8, 1932  |
| 1,919,725 | Jennison | July 25, 1933 |
| 2,400,234 | Hudson   | May 14, 1946  |

#### OTHER REFERENCES

"Aluminum Bronze," 1939 ed., page 61.  
 "Metals" by Carpenter and Robertson, vol. 2, 1939, pages 1308 and 1309.